

## UNITED STATES PATENT OFFICE

HORACE A. STAPLES, OF PLAINFIELD, NEW JERSEY, ASSIGNOR TO NATIONAL ELECTRIC PRODUCTS CORPORATION, OF NEW YORK, N. Y., A CORPORATION OF DELAWARE

## PROTECTIVE COATING AND METHOD OF PRODUCING THE SAME

No Drawing.

Application filed September 29, 1930. Serial No. 485,313.

This invention relates to improved protecting coatings for non-ferrous materials such as brass or other alloys containing copper. More particularly the invention relates 5 to an improved protective coating for brass alloy tubes, parts, plates and the like and to a method for providing tubes and other non-ferrous articles with such coatings.

The invention has for one of its objects 10 the provision of an improved protective coating for resisting corrosion which coating improves the appearance of the product, and which coating is adapted for use upon non-ferrous articles such as tubes, plates or other 15 parts formed of brass and like alloys.

A further object of the present invention resides in the provision of a novel method of obtaining the desired coating.

A further object of the present invention 20 resides in the provision of a method of coating brass alloys and like non-ferrous materials by the use of which uniformity of product may be secured at less expense than before and with less loss.

25 A further object of the present invention resides in the provision of a coating process which will enable coatings to be applied upon articles which heretofore were not readily capable of receiving coatings on account of 30 their composition or proportions and furthermore to provide a coating process which will enable proper coatings to be applied while at the same time preventing over annealing of the alloy during the formation of 35 the coating.

Further and other objects of the present invention will be hereinafter set forth in the specification and claims.

A careful study of the causes of failure of 40 brass alloy tubes in heat exchangers, condensers, etc., shows that a large percentage of failures are caused by corrosion of the surfaces subjected to the conveyed fluids. To protect these surfaces with a non-corrosive 45 substance would be ideal and very desirable for lengthening the usable tube life. Attempts have been made to accomplish these results heretofore by the use of various non-metallic compounds, but these results have 50 not met with much success because of the

lack of uniformity of the film and frequently the compounds have been of such nature as to cause considerable loss in heat transfer.

It has accordingly been appreciated that an ideal protective coating would be a metallic oxide coating. Such a coating in general is less soluble in solutions than the corresponding metal or alloy. It is also apparent that with a brass alloy tube the natural choice of a protective coating should fall 55 on cupric oxide as copper is the predominating metal in the alloy. Such a coating should be an integral part of the tube and would allow the maximum amount of heat transfer. It may be pointed out that a prolonged 60 exposure of a brass alloy to the elements produces a compact film of oxides on the alloys which is known as "weathering". The weathering effect may be greatly accelerated 65 by chemical action, also heat applied to the 70 brass alloy in the presence of air will produce oxidization of the surfaces and result in a film of oxide which in reality can be considered an integral part of metal in the tube. This chemical reaction in the case of copper 75 is illustrated by the following equations:

- (1)  $4\text{Cu} + \text{O}_2 \xrightarrow{\text{heat}} 2\text{Cu}_2\text{O}$  (red cuprous oxide)
- (2)  $2\text{Cu}_2\text{O} + \text{O}_2 \xrightarrow{\text{heat}} 4\text{CuO}$  80 (black cupric oxide)
- (3)  $2\text{Cu} + \text{O}_2 \xrightarrow{\text{heat}} 2\text{CuO}$ .

From the above equations it will be seen that the presence of insufficient oxygen produces the relatively unstable red cuprous oxide which on further oxidation becomes the black cupric oxide. The more desirable oxide coating would be the black cupric oxide coating which it has been shown can be produced by annealing brass in the presence of 85 sufficient oxygen. This process is sometimes attempted in commercial practice by leaving on the tube or other part the film of oxide produced by the final annealing operation instead of cleaning off the film with acids. At 90 attempts have also been made heretofore to accelerate this action by dipping the tubes in various compounds. It has been found, however, that it is impossible with the ordinary annealing furnaces to secure a uniform 95 100

film of oxide; in fact portions of the tube would not be covered at all. In other cases while the exteriors of the tubes were properly coated with the desired black oxide coating 5 the interiors of the tubes or portions thereof were coated with a cuprous oxide coating which coating did not provide the desired proper protection.

To attain improved degrees of perfection 10 in the applied coatings, special furnaces have been provided whereby continuous uniform heat could be applied in the presence of an excess of oxygen. Variations in the films occurred, however, even when special furnaces 15 were employed and even when previously known compounds were employed to facilitate the formation of the coating.

The application of black oxide coatings to 20 brass tubes or like non-ferrous alloy parts also in practice presents other difficulties. Such material for proper heat treatment requires the subjecting of the material to heats of varying degrees of temperature depending upon the initial hardness of the material. 25 With higher degrees of hardness after drawing or working operations, relatively lower temperatures are required for complete recrystallization, and with relatively lower degrees of hardness relatively higher temperatures are required. Time factors are also involved. If a certain time of heat treatment 30 is exceeded at a given temperature over annealing will occur and the grain structure of the alloy will become too large. Formation 35 of a black oxide requires a given temperature and the time factor to obtain a proper coating will vary with a variation of a mass of the article to be coated, because the high conductivity of the material will carry heat 40 away from the surface to be coated so that it will not oxidize as properly or as readily as it should to provide a proper coating. Furthermore, variation in the zinc content of the alloy also necessitates a variation in the 45 time factor for producing a proper coating because with material having relatively greater zinc content more material has to be removed to leave sufficient oxide to provide the proper coating. To properly oxidize the 50 material, the more time that is used for the heat treatment, the better the coating will be within certain limits. However, the time of treatment for securing the proper and desired oxide coatings will frequently exceed 55 the time permitted for heat treatment to obtain proper grain construction in the alloy.

To provide a proper and relatively uniform black oxide coating under the foregoing conditions which are to a certain extent 60 antagonistic to each other, requires a modification to the previously used process which will now be described. In lieu of first annealing the article, then immersing it in a bath of drawing compound comprised of talc, 65 soap, water and oil, then drawing the

article and subsequently annealing the tube or other part in the presence of an excess of oxygen, the process is modified by adding to the usual drawing compound a quantity of kerosene. In practice the quantity of kerosene which is used may be varied, but substantially two gallons of kerosene to fifty gallons of drawing compound provides a typical and suitable mixture. The action 70 of the kerosene in facilitating and improving the formation of a black oxide film is not entirely understood, but its use seems to accelerate the formation of the oxide upon the subsequent heat treatment and accordingly, 75 a uniform film of the desired texture and character is produced. Furthermore, with tubes the coating is uniform both inside and outside the tube and the formation of undesired red cuprous oxide coatings is obviated. 80

The use of kerosene in the drawing compound further seems in some way to accelerate the removal of the zinc from the alloy and its use brings about the formation of the oxide coating in proper time to obviate over annealing in the subsequent heat treatment. The use of kerosene also provides for the formation of coatings of desired uniform characteristics upon alloys which have so high a zinc content as to render a formation 85 of a proper black oxide coating difficult if not impossible heretofore. The use of kerosene also permits the forming of coatings upon thin wall tubes which heretofore were over annealed during the formation of 90 oxide coatings thereon.

The established practice in the art is to pickle with diluted sulphuric acid after every annealing operation. Such pickling step is necessary with non-uniform and irregular oxide formations upon the tube. However, according to the present process with some alloys the practice can be adopted of completely eliminating the customary pickling operations after annealing. In fact 100 some parts may be made with no pickling operations whatsoever. Obviously a number of drawing and oxide forming operations may be employed.

In other cases with different alloys, pickling 105 steps after annealing are retained except for the final heat treatment and coating formation step.

What I claim is:

1. The method of providing a protective coating for the surface of a copper or copper alloy article which includes the step of adding an oxidizing accelerating agent comprising kerosene to the drawing compound for accelerating the oxidation of the material, and the step of subsequently, after drawing, 120 effecting oxidation by heating the article in the presence of an excess of an oxygen.

2. The method of providing a protective corrosion resisting coating upon copper or copper alloy products such as tubing, where- 130

in oxidizing of the surface of the product is effected by a heat treatment after drawing, which includes the step of accelerating the formation of the oxidized coating and providing a uniform coating by adding kerosene to the drawing compound in which the products are immersed prior to drawing, and the step of thereafter applying such coating by an oxidizing heat treatment of the product.

10 3. A heat treated copper or copper alloy tube with proper grain structure as secured with proper annealing with an interior and exterior of corrosion-resisting black cupric oxide finish of substantially uniform character 15 inside and outside and substantially free from cuprous oxide.

4. The method of providing corrosion resisting coating upon copper or copper alloy articles which are drawn and thereafter heat treated which includes the step of improving the character of the coating and obtaining uniformity of the coating by adding a petroleum distillate such as kerosene to the drawing compound, thereafter drawing the article 25 and thereafter heat treating it in the presence of an excess of oxygen.

5. A method of providing drawn tubes and like articles of copper or copper alloy with protective coatings and for heat treating the 30 tubes or the like, which comprises coordinating the formation of the coating while maintaining the proper heat treatment of the article, by utilizing kerosene with the drawing compound in the drawing operation, for accelerating the formation of a proper and uniform coating during subsequent heat treatment, and by heat treating the article in an excess of oxygen without over-annealing.

40 6. A heat treated part formed of copper or copper alloy and having a protective black cupric oxide coating thereon over its entire surface and having its mass relations such that the part would over anneal if subjected 45 to heat treatment to provide the requisite coating, said part having the grain structure which is provided with proper annealing and having the black cupric oxide coating of uniform and corrosion-resisting character over 50 the surface of the article, said oxide being derived from the alloy itself and oxygen in the presence of heat.

7. The method of providing a protective 55 corrosion resisting coating on copper or copper alloy articles, including providing for uniformity of character and complete formation of a protective coating by working the article with a working compound containing an oxide accelerating material comprising 60 kerosene and thereafter oxidizing the surface of the article to provide a uniform oxidized coating thereon by heat treating the article in an excess of oxygen.

8. A heat treated copper or copper alloy 65 article having over its surface a uniform cor-

rosion-resisting black cupric oxide finish provided by working the article with a drawing compound including kerosene for accelerating subsequent oxidation and by thereafter heat-treating the article in the presence of 70 an excess of oxygen.

In testimony whereof I hereto affix my signature.

HORACE A. STAPLES.

75

80

85

90

95

100

105

110

115

120

125

130